

## UNITED STATES PATENT OFFICE

2,253,228

## LUBRICATING OIL COMPOSITION, INHIBITOR THEREFOR, AND METHOD OF MANUFACTURING THE SAME

Troy Lee Cantrell and James Otho Turner, Lansdowne, Pa., assignors to Gulf Oil Corporation, Pittsburgh, Pa., a corporation of Pennsylvania

No Drawing. Application September 15, 1936,  
Serial No. 100,956

12 Claims. (Cl. 252—46)

Our invention relates to lubricating oils and more particularly to lubricating oil compositions containing an oil-soluble agent or agents effective to inhibit or mitigate the normal corrosive or destructive action of lubricating oil deterioration products upon certain types of bearing metals under certain conditions of use, said agent or agents also having the properties of imparting so-called "extreme-pressure" characteristics to the lubricating oil compositions, and also being effective to reduce or eliminate undesirable oxidation changes in the oil.

Despite the many technological advances made in the art of refining and applying lubricating oils and in the composition of bearing materials, modern lubricating oils and bearings often fail to perform satisfactorily. It is well known in the art that straight petroleum lubricants have fairly well defined limits of bearing speeds, pressures, and temperatures within which they will give acceptable service. These limitations are often exceeded in modern designs, resulting in machines that cannot be satisfactorily lubricated by straight mineral oils. These modern designs are justified by engineers in their efforts to provide machines to conform to the ever-increasing demand for compactness, speed, power, and acceleration in modern engines. Many modern designs have already exceeded the above-mentioned limits wherein straight petroleum lubricating oils perform acceptably; therefore, it is necessary to provide lubricating compositions that extend and widen the limits formerly associated with straight lubricating oils.

Moreover, highly paraffinic oils having excellent viscosity-gravity constants, volatilities, carbon residue values, and resistance to sludging and oxidation, and hence of high value for use under relatively mild lubricating conditions, sometimes tend to be even less satisfactory than the less highly paraffinic oils, when the ordinary limits of temperature, pressure, and bearing speed are exceeded. This may be due in part to the fact that the deterioration products of paraffinic constituents are more active than those resulting from naphthenic or other nonparaffinic constituents, and it may be due also to the fact that the nonparaffinic constituents have some inhibiting effect upon either the deterioration of the paraffinic constituents or upon the behavior of products resulting from such deterioration, at high temperatures and pressures, and in the presence of certain metals. However, the inhibiting value of the nonparaffinic constituents

is low per unit concentration, and they are less satisfactory with respect to viscosity-gravity constant, carbon residue, and similar criteria of lubricating quality than the paraffinic constituents. A more satisfactory solution of the problem would be to substitute for the nonparaffinic constituents removed in the more drastic refining treatments or absent because of the highly paraffinic nature of the original stock, some inhibiting or mitigating agent which would be far more effective per unit concentration and hence less detrimental with respect to the other physical properties which also effect the ultimate lubricating value of the oil.

15 Improved bearing metals have recently been developed which are mechanically advantageous under many operating conditions. These bearing metals include binary and ternary alloys of cadmium, silver, copper, lead, and nickel; as examples of such improved bearing metals frequently employed at the present time we may mention cadmium-silver, cadmium-silver-copper, cadmium-nickel-copper, and copper-lead alloys. However, such alloys are more subject to chemical attack than babbitt and other bearing alloys used in the past, and their use at high temperatures, high speeds, and high pressures is sometimes accompanied by a deterioration of the oils employed for their lubrication, which in turn may destroy the bearings. The exact mechanism of this action is no doubt complicated and is perhaps not fully understood; it is quite possible that some of the metals present in the bearings tend to promote such deterioration, and that other metals present are subject to attack from the deterioration products. Whatever the cause or the mechanism, the result is that the combination of drastic lubricating conditions and alloy bearings of the general nature indicated frequently causes trouble; the bearings may be badly etched or corroded, and the quality of the oil may be rapidly deteriorated.

45 It has been observed in some cases that the more highly paraffinic oils are apt to cause more difficulty in this respect than less paraffinic oils. It is highly desirable, therefore, to provide means whereby the oils may be so improved as to give satisfactory operating results under the conditions noted, and this is especially true insofar as concerns the more highly paraffinic oils, which should and do command a premium in price.

Moreover, it is well known that all hydrocarbon oils are more or less subject to changes through oxidation resulting in undesirable deterioration,

acid formation, and increase in carbon residue, viscosity, sludging, and the like. Such oxidative changes may become more rapid or more far-reaching in extent in the presence of metals such as those employed in modern bearings, for example those of the general class mentioned above.

In order to meet these problems and to provide more satisfactory lubrication under the conditions indicated, various improvement agents have been incorporated in hydrocarbon oils prior to their sale and use. Some of these are extremely effective but too expensive for general use. Others, while having satisfactory inhibiting or mitigating characteristics, are unsatisfactory for other reasons. A primary requisite of any such improvement agents is good oil-solubility under service and marketing conditions; moreover, since solubilities vary in different types of oils, the improvement agent should be capable of being added in the requisite amount to oils of different characters.

The improvement agent should also be highly effective per unit concentration in the lubricating oil compositions; otherwise it would be necessary to add such an amount of the improvement agent as to substantially modify many of the desirable physical properties of the lubricating oil itself. The lubricating oils in which the improvement agents are incorporated have been carefully refined to meet exacting specifications, and if it is necessary to incorporate therein a relatively large amount of some agent differing in physical properties from the oil itself, the resulting composition may prove unsatisfactory for the very purposes for which the lubricating oil was prepared. In general, it is desirable that the improvement agent should be effective at concentrations not exceeding one or two per cent by weight of the lubricating oil, although somewhat higher concentrations may occasionally be justified for special purposes.

It is therefore an object of our invention to provide an improvement agent or inhibitor for addition to hydrocarbon lubricating oils which agent shall be in the form of a compound or compounds containing sulfur, or containing both phosphorus and sulfur, and having a satisfactory inhibiting or mitigating effect upon the destructive action of lubricating oils on alloy bearing surfaces under actual conditions of use where such destructive action would otherwise take place.

It is also an object of our invention to provide an improvement agent or agents of the character indicated herein, having the property of imparting desirable extreme-pressure characteristics to hydrocarbon oils when incorporated therein.

Another object of our invention comprises the provision of an improvement agent or agents for addition to hydrocarbon oils, having desirable anti-oxidant and stabilizing properties, and effective to retard increase in viscosity, carbon residue, acidity, and sludging of both highly paraffinic and less highly paraffinic oils.

A further object of our invention is to provide improved lubricating compositions comprising hydrocarbon lubricating oils and certain improvement agents incorporated therein.

A still further object of our invention is to provide a method or methods of manufacturing improvement agents having desirable characteristics for addition to mineral oils.

Our invention has for further objects such

additional operative advantages and improvements as may hereinafter be found to obtain.

We have found that extremely effective improvement agents or inhibitors of the general character indicated can be prepared by reacting sulfur chloride or a mixture of sulfur chloride and phosphorus trichloride with certain anti-oxidants, said anti-oxidants comprising water-insoluble reaction products obtained by reacting phenols with olefins. Such anti-oxidants and methods of preparing the same are disclosed in the prior copending application of Stevens and Gruse, Serial No. 702,258, filed December 13, 1933, now issued as Patent No. 2,061,111, of November 15, 1936, and in the co-pending applications of Troy Lee Cantrell, Serial No. 64,413, filed February 17, 1936, and Serial No. 99,488 filed September 4, 1936, now issued as Patent No. 2,149,759, of March 7, 1939, to which reference may be had for further details. The disclosures of the copending applications referred to constitute in effect a part of the disclosure of our present application, insofar as relates to the preparation of such anti-oxidant materials, which are used as starting materials in preparing improvement agents in accordance with our present invention. Referring, for example, to the aforesaid co-pending application, Serial No. 99,488, there is disclosed a process for the manufacture of anti-oxidant wherein a phenol is mixed with from 1 to 10 per cent of sulfuric acid having strength of 60 to 100 per cent, or even fuming sulfuric acid, and an olefin or mixture of olefins is passed, preferably in the vaporous or gaseous phase, through the liquid mixture until the phenol undergoing reaction has gained in weight from 100 to 200 per cent, or thereabouts, followed by washing the product so obtained with water and caustic soda solution, the concentration of which does not exceed 15 per cent. Various phenols may be employed, for example phenol ( $C_6H_5OH$ ) itself, the three cresols ( $C_6H_4-CH_3-OH$ ), and certain xylenols ( $C_6H_3-(CH_3)_2-OH$ ) or crude cresylic acids also may be employed. The phenolic starting material should be as free as possible from pyridine bases; such pyridine bases may be removed by conventional methods such as washing with acid, or by distillation. As olefinic material there may be employed individual olefins themselves, mixtures of olefins, or mixtures of olefinic and non-olefinic material. By way of example, the olefinic starting material may be butylenes, amylenes, refinery gases containing normally gaseous olefins (ethylenes, butylene, propylene) in varying amounts, and cracked distillates or other relatively low-boiling hydrocarbon mixtures containing normally liquid olefins and in some instances also containing substantial amounts of distilled normally gaseous olefins.

When the reaction is conducted with the olefin in the gaseous phase, the product is relatively highly concentrated with respect to effective anti-oxidant material and may not require distillation or concentration for the purpose of isolating the latter. On the other hand, when the reaction is conducted with the olefinic material in liquid phase, and especially when the concentration of olefins in the starting material is comparatively low, the product may be relatively dilute with respect to the effective anti-oxidant material, comprising for example a solution of such anti-oxidant in gasoline-like polymers or unreacted liquid hydrocarbons. In such case, the

anti-oxidant material may be concentrated by distillation or otherwise as set forth in the above-mentioned co-pending applications, prior to use in the process described herein.

The exact chemical and structural nature of the anti-oxidant materials, as thus prepared and employed as starting material in the manufacture of our improved addition agents, is largely obscure. Although we have been able to identify certain types of compounds in these anti-oxidant materials, it will be realized that, especially since mixtures of various phenols and mixtures of various olefins are frequently employed in the manufacture of these anti-oxidants, the number of possible chemical compounds is large and varied. In general, they differ from the simple alkylated phenols in that they are insoluble in dilute caustic soda solution, and also in that they are good anti-oxidants and gum-inhibitors, whereas simple alkylated phenols are not. In general, also, the alkylations, in such instances as they occur, are of secondary and tertiary types; the methods set forth in the above co-pending applications do not produce normal or primary alkylation linkages. Alkylated phenols with normal or primary linkages are undesirable, due to the fact that both such materials and their products of reaction with sulfur chloride or mixtures of sulfur chloride and phosphorus trichloride tend to be relatively insoluble in high-gravity lubricating oils. It is possible that certain alkylated phenols of normal or primary linkage might be satisfactory provided the chains were long enough, say chains of four carbon atoms or more, on account of the closer resemblance in structure of such compounds to paraffinic lubricating oil constituents. However, this is doubtful and such compounds would be expected to be of prohibitive cost.

We have identified as constituents in the various anti-oxidant materials prepared as set forth hereinbefore such compounds as follows:

Ortho-isopropyl phenol

Ortho-tertiary butyl phenol

2,4-ditertiary butyl phenol

Ortho-isoamyl phenol

Ortho-tertiary amyl phenol

In addition to the above-listed compounds, similar derivatives of various homologues of mono-, di-, and poly-hydroxy phenols may be present. It may be remarked, however, that while some of the constituents of such anti-oxidants may be identified, it is difficult or impossible to identify all of the constituents of any one anti-oxidant material of the character indicated and it is equally impossible to say which particular compound or type of compound may be the most important. As a matter of fact, we have not been able to isolate or identify any single constituent or to recover any fraction of the concentrated anti-oxidants prepared in accordance with the aforesaid Cantrell application, Serial No. 99,488, which constituent or fraction has an anti-oxidant value as high as that of the total concentrated product. Nor for the purpose of our present invention is it necessary so to do; the fact remains that anti-oxidants may be prepared in the manner set forth hereinbefore and in the aforesaid co-pending applications, and such materials comprise suitable starting materials for the manufacture of sulfur-containing improvement agents or inhibitors in accordance with our present invention; certain of the constituents of the anti-oxidant starting material

which are not in themselves effective as anti-oxidants are nevertheless capable of being converted by reaction with sulfur chloride or a mixture of sulfur chloride and phosphorus trichloride to sulfur-containing materials useful as inhibitors. As aforesaid, we prepare our improved addition agents or inhibitors by reacting anti-oxidants of the general character described herein with sulfur chloride alone or with a mixture of sulfur chloride and phosphorus trichloride. We may also treat one batch of anti-oxidant material with  $S_2Cl_2$  and another batch with  $PCl_3$  and blend the products. In this case, however, the results are not necessarily identical with those prepared by using a mixture of  $S_2Cl_2$  and  $PCl_3$ , because of the possibility of interreaction between the latter, prior to and during the reaction with the anti-oxidant. For example, the following reaction may take place at a temperature of 160° F. or higher:  $3PCl_3 + S_2Cl_2 \rightarrow PCl_5 + 2PSCl_3$ . The  $PCl_5$  and  $PSCl_3$  resulting from this reaction, if it occurs, will in turn react with the anti-oxidant; the products of the latter reaction are obviously not the same compounds as those resulting from individual and separate reactions with  $S_2Cl_2$  and  $PCl_3$ , respectively, but they are also effective and useful for the purposes to which our invention is addressed.

The general procedure is as follows: The anti-oxidant material, which preferably should be dry, is mixed either at atmospheric temperature or at a slightly elevated temperature with sulfur chloride or a mixture of sulfur chloride and phosphorus trichloride, the mixture being stirred as the reaction proceeds. The temperature is then raised to 300° F., or thereabouts, and maintained at this elevated temperature for a suitable time in order to drive off hydrogen chloride resulting from the reaction. The product is then cooled and may be used as such, although it is nearly always desirable to decolorize it, to some extent at least. Thus the product may be cooled to around 250° F., and treated at that temperature with a suitable solid absorbent material such as fuller's earth, charcoal, acid-treated clay or the like. Alternatively the inhibitor, after cooling to atmospheric temperature, may be diluted with a suitable hydrocarbon liquid of lower viscosity in preparation for the filtration step. By way of example, we may employ a light naphtha as a diluent; the use of naphtha has the advantage that such naphtha may be removed after the decolorizing operation by distillation. Or we may employ as diluent a low-viscosity lubricating oil similar to the oil to which the inhibitor is eventually to be added; in such case it is unnecessary to remove the diluent prior to incorporating the inhibitor in the lubricating oil.

The amount of reagent added will vary over a considerable range, depending upon the desired characteristics of the final product and the degree of concentration of the anti-oxidant. Where the anti-oxidant starting material is relatively highly concentrated and the reagent or reagents are added in sufficient amount to react fully with all of the anti-oxidant present, the products tend to be of high viscosity. With sulfur chloride alone we have prepared products containing as much as 10 per cent by weight of sulfur, and fairly effective materials containing as little as 1 per cent by weight of sulfur. However, we find that the best results are obtained by limiting the amount of sulfur chloride added to give products containing from about 5 to 7 per cent

of sulfur, assuming the anti-oxidant starting material to be free or relatively free from diluent. Products containing sulfur within this preferred range are effective enough to be economical, and their physical properties such as solubility in oil, viscosity, and color make them highly suitable as addition agents, especially for incorporation in highly paraffinic oils. Moreover, by limiting the amount of sulfur chloride added to a point short of completion of reaction with all of the anti-oxidant, we obtain final products comprising mixtures of the sulfur-containing inhibitor and some of the original anti-oxidant material and having exceptionally advantageous properties. The unreacted anti-oxidant serves as a blending agent and also contributes anti-oxidant and stabilizing properties, so that the products thus prepared are very soluble in highly paraffinic oils and while effective as inhibitors also have high anti-oxidant and stabilizing value, and are themselves stable to an advantageous extent.

In employing a mixture of sulfur chloride and phosphorus trichloride, or in blending the products separately prepared by reacting sulfur chloride and phosphorus trichloride, respectively, with anti-oxidant material of the character indicated, the total amount of combined sulfur and phosphorus should not exceed about ten per cent by weight of the final product. The preferred products are those which contain from 1.0 to 3.0 per cent of phosphorus and from 1.0 to 5.0 per cent of sulfur. As in the case of reaction with sulfur chloride alone, advantageous results may be secured by limiting the amounts of sulfur chloride and phosphorus trichloride to a point short of completion of the reaction with all of the anti-oxidant present.

We prefer to employ as starting materials anti-oxidants, prepared as set forth above and in the aforesaid co-pending applications, and having physical properties within the following range:

|                                     |                           |
|-------------------------------------|---------------------------|
| Gravity, °API.....                  | 15.0 to 25.0              |
| Specific gravity; 60°/60° F.....    | 0.9659 to 0.9042          |
| Viscosity, SUV at 100° F.....       | 150 to (solid)            |
| Color.....                          | Water white<br>to 7 (NPA) |
| Pour point (liquids only) °F.....   | 0 to 30                   |
| Melting point (solids only) °F..... | 80 to 225                 |

Our invention, in its broadest aspects, however, is not limited to the preferred starting material mentioned hereinabove but contemplates the manufacture of inhibitors of the general class described from any alkylated phenols so long as such alkylated phenols possess definite anti-oxidant properties, are insoluble in water, insoluble or only slightly soluble in dilute alkali, and are permanently soluble up to 5 per cent in paraffin oils. For example, we may employ as starting materials anti-oxidants prepared by reacting various light cracked hydrocarbon distillates and other normally liquid olefinic mixtures with phenol, as described in the aforesaid co-pending applications. It is a requisite of such olefin-phenol reaction products, however, insofar as the present process is concerned, that compounds contained therein shall contain one or more secondary or tertiary carbon linkages or both.

The anti-oxidant value of this starting material should be such that the addition of 0.01 per cent by weight thereof to standard gasoline stock having an oxygen stability test (E. G. C. meth-

od) of, say, 120 minutes, will raise the oxygen stability to at least 240 minutes. Less potent anti-oxidants are unsuitable as starting materials.

5 The character of the final sulfur-containing inhibitor will, of course, vary with the character of the phenolic and olefinic material employed in the manufacture of the anti-oxidant starting material, with the extent of absorption of the olefin, and with the amount of sulfur, or phosphorus and sulfur, subsequently introduced. All of these factors are very intimately inter-related. These are the primary factors, but it will be obvious that there are numerous secondary factors, 10 for example the degree of purification and decolorization of the anti-oxidant starting material.

Naturally, it is to be expected that the viscosities, specific gravities and other physical 15 characteristics of the particular phenol employed will have a corresponding effect upon the product, to some extent at least; this effect may, however, not always hold true where the degree of olefin absorption varies over comparatively wide 20 limits and where the percentage of sulfur, or of phosphorus and sulfur, in the final compound also varies.

When cresylic acid, ortho-cresol and meta-cresol and the like are used in the manufacture 25 of the anti-oxidant, we prefer to limit the olefin absorption to around one mol per mol of the phenolic material, i. e., to give a water-insoluble product representing roughly 135 to 150 per cent by volume of the original phenol, in order ultimately to secure inhibitors that are sufficiently 30 soluble in the higher gravity oils.

When the anti-oxidant starting material is 35 prepared from phenol ( $C_6H_5OH$ ) itself, e. g., "90 per cent phenol," the degree of absorption of 40 olefin may be carried farther, for example to about two mols of olefin per mol of phenol (based on the assumption that the olefin is made up entirely of  $C_4$  hydrocarbons).

The preferred olefins are those containing 45 from three to eight carbon atoms per molecule; the higher the molecular weight of the olefin, the more viscous the final product will be. Olefins containing more than eight carbon atoms per molecule tend to reduce the sulfur content 50 of the final inhibitor product. Ethylene ( $C_2H_4$ ), on the other hand, is insufficiently reactive, requiring the use of fuming sulfuric acid, and does not sufficiently reduce the activity of the original phenol.

55 The best olefin starting materials are those containing from three to five carbon atoms per molecule, especially butylenes; fractions obtained from gases produced in the pyrolysis of hydrocarbon oils and rich in olefins of this approximate range represent advantageous and available raw materials.

After the reaction between the phenol and olefin has been carried to the desired degree of 60 completion, the product is washed with water and dilute caustic soda in the manner set forth hereinabove and in the aforesaid co-pending applications. The resultant water-insoluble anti-oxidant material is then preferably dried. The 65 drying may be accomplished by filtering the material through absorbent clay or the like, the effect of which is to dehydrate and decolorize. Or, the drying may be accomplished by heating the anti-oxidant material to about 400° F. in 70 suitable apparatus; this procedure dehydrates

and tends to darken the anti-oxidant material.

The dry anti-oxidant may then be treated directly with the reagent or reagents, or it may first be distilled to separate undesirable low-boiling and high-boiling constituents, respectively. Thus we may distill under a vacuum of from -11 in. to -28 in. Hg, to recover a fraction distilling over between 300° and 550° F., which fraction may then be treated with sulfur chloride, or a mixture of sulfur chloride and phosphorus trichloride. The lower boiling material, and sometimes also the residue, may be recycled for further reaction with olefins in the presence of sulfuric acid, or used as an anti-oxidant.

The following examples will serve to illustrate our invention in some of its more specific embodiments.

EXAMPLE 1

(a) Preparation of anti-oxidant starting material

20 gals. of "90 per cent phenol" were mixed with 5 per cent by weight of 94.5% sulphuric acid (C. P.). Olefin gas composed primarily of C<sub>4</sub> hydrocarbons was then introduced into close contact with the phenol-acid mixture until the volume of the reacting mixture increased to about 45 gals. This product was washed with 10 gals. of 15% caustic soda and later with 10 gals. of water. After neutralization the recovered product amounted to about 40 gals. Typical properties of anti-oxidant material prepared in this manner are as follows:

Gravity, °API..... 22.4  
Viscosity, SUV, seconds:  
    100° F..... 180  
    210° F..... 37.6  
Pour point, °F..... +15

(b) Preparation of final inhibitor

To 88 parts by weight of the anti-oxidant material prepared as described above, and preferably dry, 12 parts by weight of sulfur chloride were slowly added, the temperature meanwhile being raised to about 300° F. and held at that temperature until evolution of hydrogen chloride ceased. The reaction product was then cooled to about 250° F., and was decolorized by contact with acid-treated clay. The resulting product had the following properties:

Gravity, °API..... 12.4  
Viscosity, SUV at 100° F., seconds..... 1635  
Color, NPA..... 6  
Sulfur, percent by weight..... 6.35

This product is a viscous, oil-like material resembling dark motor oil in appearance. (It will be obvious that the color of the material prepared in this manner will vary with the extent of decolorization.) It is a highly suitable improvement agent or inhibitor for incorporation in hydrocarbon oil in proportions varying from 0.25 to 1.0, or more, per cent by weight.

EXAMPLE 2

(a) Preparation of anti-oxidant starting material

Anti-oxidant material prepared as described in connection with Example 1(a), was distilled under vacuum of 11 to 12 in. Hg. The distillate was cut into three fractions. That fraction dis-

tilling over at vapor temperatures between 300° and 550° F., had the following properties:

5 Gravity, °API..... 16.8  
Viscosity, SUV at 100° F., sec..... 185  
Color, NPA..... -13

(b) Preparation of final inhibitor

82 parts by weight of an anti-oxidant fraction prepared as described above were treated with 18 parts by weight of an approximately 25:75 mixture of sulfur chloride and phosphorus trichloride, the operating procedure being that described in connection with Example 1. The resulting material had the following properties:

10 Gravity, °API..... 10.6  
Viscosity, SUV at 100° F., sec..... 731  
Color, NPA..... 1.25  
20 Phosphorus, percent by weight..... 2.10  
Sulfur, percent by weight..... 1.88

This product is much less viscous than that prepared in accordance with Example 1, and represents an extremely effective improvement agent or inhibitor for addition to hydrocarbon oils in amounts up to from 1 to 2 per cent by weight of the oil.

These inhibitors, when added to hydrocarbon oils, strongly inhibit corrosion of metal alloy 30 bearings such as those of silver, cadmium, copper and nickel, under conditions where the oil alone would cause such corrosion; oil compositions containing them also exhibit marked extreme-pressure characteristics. These inhibitors are 35 stable at ordinary temperatures and do not tend to deposit out of lubricating oil compositions containing them on metal surfaces such as those of tin plate, terne plate or the like when packaged and stored prior to sale and use. They are 40 permanently soluble in hydrocarbon oils of high paraffinicity. Moreover, these inhibitors have excellent anti-oxidant properties, the anti-oxidant properties rising in proportion to the amount of unreacted anti-oxidant starting material remaining in the final product. They are 45 not subject to hydrolysis to any detrimental extent; the products of such hydrolysis as may occur are in themselves anti-oxidant and non-corrosive materials.

50 In actual use, oil compositions containing our inhibitors may tend to diminish somewhat in sulfur content, a circumstance which may be accompanied by liberation of sulfur in some form, probably as hydrogen sulfide. However, this is not detrimental and may in fact be advantageous.

In preparing these materials we select or regulate the character and molecular weight of the phenolic starting material and of the olefinic starting material, respectively, the degree of 55 olefin absorption in the phenolic reaction mixture and the relative amounts and proportions of the sulfur chloride, of the mixture of sulfur chloride and phosphorus trichloride, in accordance with the final concentration and proportions of sulfur and phosphorus desired in the final product. This regulation makes it possible to secure inhibitors having desired temperature responsiveness, activity, solubility, viscosity, and color, varying closely over a wide range.

An advantage of our process and product resides in the fact that the principal ingredients employed in the manufacture of the final product, namely olefins, are cheap and available to the refiner.

The following tables will serve to illustrate the effectiveness of our inhibitors and the value of lubricating compositions containing them.

Table I

|                                       | Untreated oil | Oil containing one inhibitor (prepared as in Example 1) |
|---------------------------------------|---------------|---------------------------------------------------------|
| Make-up, percent by wt.:              |               |                                                         |
| Lubricating oil.....                  | 100           | 99.5                                                    |
| Inhibitor.....                        |               | 0.5                                                     |
| General properties:                   |               |                                                         |
| Gravity, °API.....                    | 32.5          | 32.4                                                    |
| Specific gravity, 60°/60° F.....      | 0.8268        |                                                         |
| Viscosity, S.U.V.—                    |               |                                                         |
| 100° F.....                           | 183.6         | 183.5                                                   |
| 210° F.....                           | 46.0          | 46.2                                                    |
| Viscosity index.....                  | 107.0         | 108.0                                                   |
| V-G constant.....                     | 0.804         | 0.804                                                   |
| Flash, OC: °F.....                    | 410           | 400                                                     |
| Fire, OC: °F.....                     | 470           | 465                                                     |
| Pour point, °F.....                   | 0             | +5                                                      |
| Color, N.P.A.....                     | 1.5           | 1.75                                                    |
| Sulfur, B: percent.....               | 0.04          | 0.10                                                    |
| Carbon residue, percent.....          | 0.04          | 0.03                                                    |
| Almen test:                           |               |                                                         |
| Lever load, lb.....                   | 10            | 16                                                      |
| Rubbing speed, ft./min.....           | 40            | 40                                                      |
| Unit load, lb./sq. in.....            | 5000          | 8000                                                    |
| Lubricant temp., °F.—                 |               |                                                         |
| Initial.....                          | 83            | 92                                                      |
| Final.....                            | 100           | 148                                                     |
| Special oxidation and corrosion test: |               |                                                         |
| Time oxidized, hr.....                | 48            | 48                                                      |
| Oil bath temperature, °F.....         | 347           | 347                                                     |
| Air rate, cc. per hr.....             | 2000          | 2000                                                    |
| Quantity of oil, cc.....              | 300           | 300                                                     |
| Oxidized oil—                         |               |                                                         |
| Gravity, °API.....                    | 30.9          | 31.6                                                    |
| Viscosity, S.U.V.—                    |               |                                                         |
| 100° F.....                           | 225.2         | 191.0                                                   |
| 210° F.....                           | 48.5          | 46.6                                                    |
| Viscosity index.....                  | 102.0         | 101.0                                                   |
| Carbon residue, percent.....          | 0.51          | 0.15                                                    |
| Neutralization No.....                | 1.82          | 0.30                                                    |
| Cadmium-silver bearing—               |               |                                                         |
| Weight before test, g.....            | 37.1833       | 36.0566                                                 |
| Weight after test, g.....             | 36.4931       | 36.0658                                                 |
| Change in weight.....                 | -0.6952       | +0.0092                                                 |
| Appearance.....                       | Etched        | Good                                                    |

Table II

|                                       | Untreated oil | Oil containing one inhibitor (prepared as in Example 2) |
|---------------------------------------|---------------|---------------------------------------------------------|
| Make-up, percent by weight:           |               |                                                         |
| Lubricating oil.....                  | 100.0         | 99.0                                                    |
| Inhibitor.....                        |               | 1.0                                                     |
| General properties:                   |               |                                                         |
| Gravity, °API.....                    | 32.5          | 32.3                                                    |
| Specific gravity, 60°/60° F.....      | 0.8268        | 0.8644                                                  |
| Lb./Gal., 60° F.....                  | 7.184         | 7.198                                                   |
| Viscosity, S.U.V.—                    |               |                                                         |
| 100° F.....                           | 186.0         | 186.0                                                   |
| 210° F.....                           | 46.1          | 46.0                                                    |
| Viscosity index.....                  | 104           | 102                                                     |
| V-G Constant.....                     | 0.804         | 0.806                                                   |
| Flash, OC: °F.....                    | 410           | 405                                                     |
| Fire, OC: °F.....                     | 465           | 475                                                     |
| Pour point, °F.....                   | 0             | 0                                                       |
| Color, N.P.A.....                     | 1.5           | 1.5                                                     |
| Sulfur, B: percent.....               | 0.04          | 0.06                                                    |
| Phosphorus, percent.....              |               | 0.02                                                    |
| Carbon residue, percent.....          | 0.05          | 0.06                                                    |
| Special oxidation and corrosion test: |               |                                                         |
| Time oxidized, hr.....                | 48            | 48                                                      |
| Oil bath temperature, °F.....         | 347           | 347                                                     |
| Air rate, cc. per hr.....             | 2000          | 2000                                                    |
| Quantity of oil, cc.....              | 300           | 300                                                     |
| Oxidized oil—                         |               |                                                         |
| Gravity, °API.....                    | 31.2          | 32.3                                                    |
| Viscosity, S.U.V.—                    |               |                                                         |
| 100° F.....                           | 210           | 191                                                     |
| 210° F.....                           | 47            | 46                                                      |
| Viscosity index.....                  | 95            | 97                                                      |
| Carbon residue, percent.....          | 0.36          | 0.18                                                    |
| Neutralization No.....                | 1.33          | 0.58                                                    |
| Cadmium-silver bearing—               |               |                                                         |
| Weight before test, g.....            | 37.2149       | 36.8846                                                 |
| Weight after test, g.....             | 36.9665       | 36.8870                                                 |
| Change in weight, g.....              | -0.2484       | +0.0034                                                 |
| Appearance.....                       | Etched        | Good                                                    |

The lubricating oil used in the tests given in the tables given hereinabove was an SAE 10

grade oil which had been previously treated with aluminum chloride.

The "Special oxidation and corrosion test" referred to in the foregoing tables is conducted as follows: An alloy bearing shell of certain commonly used standard dimensions is submerged in 300 cc. of the oil or oil composition in a 400 cc. Pyrex beaker and heated in a thermostatically controlled oil bath to 175° C. (347° F.), and air, at the rate of 2000 cc. per hour, is bubbled through the oil in contact with the bearing shell. At the end of 48 and 96 hours, the loss of weight and the condition of the bearing shell are determined, the bearing shell being washed free of oil and dried before weighing. When determining the effectiveness of various improvement agents, the usual procedure is to run a "blank" test simultaneously with the oil composition being tested, employing for that purpose a sample of the untreated oil.

In this test it is advantageous to employ commercial bearing shells. These shells comprise a suitable metal backing faced with the alloy bearing metal. In this way, the actual bearing face is subjected to severe deterioration conditions. By comparison of the results of such tests with actual service tests, we have found them to be in substantial agreement as to the suitability of particular lubricants.

In the tests given in the foregoing tables we employ so-called "cadmium-silver" bearings of the following approximate composition:

| Metal        | Percent |
|--------------|---------|
| Cadmium..... | 98      |
| Silver.....  | 1       |
| Copper.....  | 1       |

In these tests the loss in weight, while not extremely high when expressed as "per cent loss," is nevertheless very significant, as the bearing shells used have an alloy facing of only 0.008 to 0.012 in. thickness on a highly resistant backing and the observed losses in the reported tests often represent a loss of the order of 10 per cent of the alloy facing.

Various modifications in the operating procedure mentioned hereinabove will suggest themselves to those skilled in the art. For example, we have described washing the phenol-olefin reaction product with water and dilute caustic soda solution to effect neutralization and removal of the acid or acids (e. g. sulfuric acid and sulfonic acids) remaining the reaction mixture after the introduction of the olefins has been discontinued. Such neutralization and removal may be effected in other ways, as by extraction with aqueous alcohol, contact with solid alkalies such as lime or sodium carbonate, or by contacting the reaction mixture with solid adsorbents such as fuller's earth, activated carbon, or the like.

Wherever the expression "highly paraffinic oil" is employed herein and in the claims herein-after made it is in general intended to indicate lubricating oils conforming in physical properties to oils prepared from Pennsylvania crudes; these "highly paraffinic oils" are either oils derived from Pennsylvania crudes or oils which have been refined or blended to approach or even exceed the latter oils in paraffinicity. Where various materials are referred to as being soluble in such paraffinic oils, this expression is intended to mean that such materials may be incorporated into such oils in amounts up to 10 per cent, with-

out producing any haziness nor cloudiness in the appearance of the resultant compositions, at least under atmospheric temperatures and under the ordinary conditions to which such oil compositions are subjected in storage and handling prior to their actual use as lubricants.

In referring to "sulfur chloride" herein, we intend to designate any of the various chlorides of sulfur. The preferred compound is  $S_2Cl_2$ ; however, commercial grades of this compound may contain varying quantities of other chlorides of sulfur such as  $SCl_2$ ,  $S_3Cl_4$ ,  $SCl_4$ , and  $S_3Cl_2$ . We may employ as the sulfur-containing reagent any of these sulfur chlorides, or mixtures of any two or more of the same.

While we have described our invention hereinabove with reference to various preferred forms and embodiments, and with reference to various specific examples, it will be understood that our invention is not limited to the details of such illustrative embodiments or examples but may be variously practiced and embodied within the scope of the claims hereinafter made. Moreover, while we have in certain instances specifically given certain preferred ranges and proportions, it will be understood that our invention is not limited thereto and that such preferred ranges and proportions are in general selected for particular products and particular purposes; variations in proportions and in the methods of preparation result in products of different characteristics, such products having individual advantages and utilities.

What we claim is:

1. The method of preparing an oil-soluble organic sulfur compound suitable as an improvement agent for hydrocarbon oils, which comprises reacting a sulfur chloride with a water-insoluble reaction product of a phenol and an olefin having anti-oxidant properties when added to a hydrocarbon oil, the reaction being carried to such extent as to incorporate sufficient sulfur into the final product to give the final product the property of inhibiting the corrosion of bearing metals by hydrocarbon oil, when added to such oil, while retaining to a substantial extent the anti-oxidant value of the aforesaid phenol-olefin reaction product.

2. The method of preparing an oil-soluble organic sulfur compound suitable as an improvement agent for hydrocarbon oils, which comprises passing a gaseous olefin into contact with a phenol in the presence of sulfuric acid until the reacting mixture has increased in volume from 30 to 250 per cent on the original phenol, neutralizing the resultant anti-oxidant product, and reacting at least a portion of the neutralized water-insoluble anti-oxidant product with a sulfur chloride to obtain a final oil-soluble material containing not more than about 7 per cent of sulfur.

3. The method of preparing an oil-soluble organic sulfur compound suitable as an improvement agent for hydrocarbon oils, which comprises passing a gaseous olefin into contact with a phenol in the presence of a catalyst until the phenol has absorbed from one to two mols of olefin per mol of phenol, washing the resultant anti-oxidant product with water and dilute alkali, and reacting at least a portion of the washed anti-oxidant product with a sulfur chloride.

4. An improvement agent for hydrocarbon lubricating oils comprising a sulfur-chloride reaction product of an alkylated phenol, said

alkylated phenol being a reaction product of an olefin and a phenol and a compound within the class consisting of secondary and tertiary alkylated phenols insoluble in water and in dilute alkali solution.

5. A method of lubricating bearing surfaces which comprises maintaining between bearing surfaces, one of which is an alloy of the class consisting of binary and ternary alloys of cadmium, silver, nickel, copper and lead, a film of lubricating oil which initially produces an effective lubricating action but which would normally tend to corrode the aforesaid alloy, and maintaining the effectiveness of the lubricating oil by incorporating therein a sulfur-chloride treated water-insoluble secondary or tertiary alkylated phenol in a small but sufficient proportion substantially to reduce the corrosion.

6. The method of preparing oil-soluble organic compounds suitable as improvement agents for highly paraffinic lubricating oils which comprises reacting an olefin and a phenol in the presence of a catalyst, washing the resultant product with water and dilute alkali, treating at least a portion of the product with a sulfur chloride, and regulating the degree of absorption of olefin in the initial reaction stage with reference to the specific chemical character of the phenol and olefin, to secure an intermediate water-insoluble product which, when treated in the subsequent reaction stage with the sulfur chloride in the required amount to introduce from one to seven per cent of sulfur into the aforesaid intermediate product, will yield a sulfur-containing product soluble in highly paraffinic oil.

7. The method of preparing an oil-soluble organic compound suitable as an improvement agent for highly paraffinic lubricating oils, which comprises reacting an olefin and a phenol in the presence of a catalyst, washing the resultant product with water and dilute alkali, treating a portion of the product with sulfur chloride and treating a second portion with phosphorus trichloride, and blending the resultant products to obtain a final product soluble in highly paraffinic oil, and containing a total of not more than about 10 per cent of combined sulfur and phosphorus.

8. The method of preparing an oil-soluble organic compound suitable as an improvement agent for hydrocarbon oils, which comprises reacting an olefin and a phenol in the presence of sulfuric acid, and treating at least a portion of the resultant product with a mixture of sulfur chloride and phosphorus trichloride.

9. The method of preparing an oil-soluble organic compound suitable as an improvement agent for hydrocarbon oils, which comprises reacting an olefin and a phenol in the presence of sulfuric acid, and treating at least a portion of the resultant product with a mixture of sulfur chloride and phosphorus trichloride to obtain a final inhibitor product containing a total of from about 2 to 10 per cent of combined sulfur and phosphorus.

10. The method of preparing an oil-soluble organic compound suitable as an improvement agent for hydrocarbon oils, which comprises reacting a mixture of sulfur monochloride and phosphorus trichloride with a water-insoluble reaction product of a phenol and an olefin, said reaction product having anti-oxidant properties when added to a hydrocarbon oil.

11. The method of preparing an oil-soluble

organic compound suitable as an improvement agent for hydrocarbon oils, which comprises reacting sulfur monochloride and phosphorus trichloride with water-insoluble reaction products of phenolic and olefinic materials, said reaction products having anti-oxidant properties when added to hydrocarbon oil, the reaction being carried to such extent as to incorporate sufficient phosphorus and sulfur into the final product to give the final product the property of inhibiting corrosion of bearing metals by hydrocarbon oil, when added to such oil, while retaining to a substantial extent the anti-oxidant

value of the aforesaid phenol-olefin reaction products.

5 12. A lubricating composition comprising a major amount of a hydrocarbon lubricating oil and a minor amount of a sulfur-chloride reaction product of an alkylated phenol, said alkylated phenol being a reaction product of an olefin and a phenol and a compound within the class consisting of secondary and tertiary 10 alkylated phenols insoluble in water and in dilute alkali solution.

TROY LEE CANTRELL.  
JAMES OTHO TURNER.